

# UNITED STATES PATENT OFFICE.

ROSWELL ENOS, OF WOODSTOCK, ILLINOIS.

## IMPROVEMENT IN TANNING.

Specification forming part of Letters Patent No. **11,325**, dated July 18, 1854.

*To all whom it may concern:*

Be it known that I, ROSWELL ENOS, of Woodstock, in the county of McHenry and State of Illinois, have invented a new and useful Improvement in the Process of Tanning Sole-Leather; and I do hereby declare that the following is a full and exact description thereof.

The nature of my invention consists in producing solid sole-leather in an unusually short time by commencing the tanning operation upon the sides by the use of a salted infusion of sumac and then completing said operation by the repeated use of the strongest oak or hemlock-bark liquors, substantially as hereinafter set forth.

The hair is first removed from the hides in any usual manner, and they should be thoroughly cleansed in either pure water or in a solution of salt and water. A batch of, say, fifty sides should be treated in the following manner, viz: Place the hides in a liquor composed by steeping forty pounds of Sicily sumac or one hundred and fifty pounds of unground native sumac in two hundred and fifty gallons of water and adding twenty-five pounds of salt thereto. Allow the sides to remain in said liquor from twelve to twenty-four hours, the length of time depending upon the temperature of the said liquor and the condition of the sides. About blood-heat I consider the best temperature for the aforesaid liquor. After the sides have remained the aforesaid length of time in the salted infusion of sumac the liquor should be strengthened by adding there-

to somewhere about two hundred gallons of strong oak or hemlock liquor and fifteen pounds of salt, and the sides be allowed to remain in the strengthened liquor for the space of from twelve to twenty-four hours. The sides should then be withdrawn from the above-mentioned liquor and placed in about the same quantity of a strong cold oak or hemlock liquor containing twenty pounds of salt in solution, and be allowed to remain in it for five or six days. The sides should then be withdrawn from the aforementioned cold liquor and be placed in the same quantity and quality of liquor, save that it should be of about blood-warm temperature and be allowed to remain therein five or six days, which latter operation should be repeated for six or seven times, when the sides will generally be found to be completely tanned.

While passing through each stage of my said tanning process the sides should be repeatedly handled, as all tanners are fully aware.

What I claim as my invention in the production of sole-leather, and desire to secure by Letters Patent, is—

Commencing the tanning operation upon the sides by the use of a salted infusion of sumac, and then completing said tanning operation by the repeated use of the strong oak or hemlock bark liquors, substantially as herein set forth.

ROSWELL ENOS.

Witnesses:

Z. C. ROBBINS,  
J. S. BROWN.